# EUROPEAN PATENT SPECIFICATION

(11) **EP 0 895 792 B1**
(45) Date of publication and mention of the grant of the patent: **11.06.2003**
(21) Application number: 98306349.6
(22) Date of filing: 07.08.1998
(51) Int. Cl.: A63B 37/00

(54) **Multi-piece solid golf ball**
Mehrteiliger, fester Golfball
Balle de golf solide en plusieurs pièces

(30) Priority: 08.08.1997 JP 22760897; 22.10.1997 JP 30797097
(43) Date of publication of application: 10.02.1999
(73) Proprietor: BRIDGESTONE SPORTS CO., LTD., Tokyo (JP)
(72) Inventor: Higuchi, Hiroshi, Bridgestone Sports Co., Ltd., Chichibu-shi, Saitama-ken (JP)
(74) Representative: Whalley, Kevin

(56) References cited:
- EP-A- 0 633 043
- EP-A- 0 637 459
- WO-A-97/18861
- GB-A- 2 302 546
- US-A- 4 919 434
- US-A- 5 026 067
- US-A- 5 439 227

## Description

This invention relates to a multi-piece solid golf ball comprising a solid core enclosed with a cover having an inner and an outer layer.

Golf balls of various structures have recently been proposed. In particular, many proposals were made on solid golf balls, inter alia, multi-piece solid golf balls comprising a solid core enclosed with a cover of plural layers from the standpoints of flight distance, control (or spin rate), and feeling (see US-A-4 919 434, JP-A 244174/1992, 142228/1994, 24084/1995, 24085/1995, and 10358/1997).

Nevertheless, there is a desire to have a multi-piece solid golf ball having further improved flight performance, superior spin property, and good feeling upon wood, iron and putter shots as well as good scraping resistance and durability.

Making extensive investigations to meet the above desire, we have found that it is effective for a multi-piece solid golf ball comprising a solid core and a cover of two inner and outer layers surrounding the core that the solid core is formed relatively soft, the inner cover layer is formed mainly of a thermoplastic polyester elastomer, the outer cover layer is formed mainly of a thermoplastic polyurethane elastomer, the inner cover layer has a Shore D hardness of 28 to 58, and the outer cover layer has a Shore D hardness of 30 to 55.

Specifically, the present invention provides:
(1) A multi-piece solid golf ball comprising a solid core and a cover having an inner and an outer layer surrounding the core, characterized in that said solid core has a distortion of at least 2.7 mm under an applied load of 100 kg, said inner cover layer is formed mainly of a thermoplastic polyester elastomer, said outer cover layer is formed mainly of a thermoplastic polyurethane elastomer, one or more ionomer resins having a Shore D hardness of at least 55 are mixed with either one or both of the thermoplastic polyester elastomer of said inner cover layer and the thermoplastic polyurethane elastomer of said outer cover layer, said inner cover layer has a Shore D hardness of 28 to 58, and said outer cover layer has a Shore D hardness of 30 to 55.
(2) The golf ball of (1) having the inner cover layer wherein the ionomer resin having a Shore D hardness of at least 55 is mixed in a proportion of 3 to 70 parts by weight per 100 parts by weight of the thermoplastic polyester elastomer.
(3) The golf ball of (1) or (2) having the outer cover layer wherein the ionomer resin having a Shore D hardness of at least 55 is mixed in a proportion of 2 to 70 parts by weight per 100 parts by weight of the thermoplastic polyurethane elastomer.
(4) The golf ball of any one of (1) to (3) wherein the ball as a whole has an inertia moment of at least 83 g-cm².
(5) The golf ball of any one of (1) to (4) wherein 0.5 to 30% by weight of an inorganic filler is added to said outer cover layer.
(6) The golf ball of any one of (1) to (5) wherein said inner cover layer contains 0 to 30% by weight of an inorganic filler.
(7) The golf ball of any one of (1) to (6) wherein said outer cover layer has a specific gravity of 1.05 to 1.4.
(8) The golf ball of any one of (1) to (7) wherein said inner cover layer has a specific gravity of 1.05 to 1.3.
(9) The golf ball of any one of (1) to (8) wherein said core has a specific gravity of 0.9 to 1.2.
(10) The golf ball of any one of (1) to (9) wherein said outer cover layer has a gage of 0.5 to 2.5 mm, said inner cover layer has a gage of 0.5 to 3.0 mm, and said cover has a total gage of 1.0 to 5.5 mm.

The golf ball of the invention features an increased flight distance, superior control upon iron shots, good feeling upon shots with any club of wood, iron and putter, high resistance to scraping upon control shots with an iron, and good durability.

Now the invention is described in more detail.

The multi-piece solid golf ball of the invention has a solid core and a cover surrounding the core of a two-layer structure of inner and outer cover layers.

The solid core used herein is formed mainly of a rubber base. Natural rubber and/or synthetic rubber which is used in conventional solid golf balls can be used as the rubber base although 1,4-polybutadiene having at least 40% of a cis structure is especially preferred in the practice of the invention. Herein, natural rubber, polyisoprene rubber, styrene-butadiene rubber or the like may be blended with the polybutadiene rubber if desired.

More particularly, the solid core of the golf ball according to the invention is obtained in conventional ways by adjusting vulcanizing conditions and blending ratio. In general, the solid core composition contains a base rubber, a crosslinking agent, a co-crosslinking agent, an inert filler, etc. The base rubber used may be the above-mentioned natural rubber and/or synthetic rubber. The crosslinking agent is exemplified by organic peroxides such as dicumyl peroxide and di-t-butyl peroxide, with the dicumyl peroxide being especially preferred. The amount of the crosslinking agent blended is usually 0.5 to 2.0 parts by weight per 100 parts by weight of the base rubber.

The co-crosslinking agent is not critical and exemplified by metal salts of unsaturated fatty acids, especially zinc and magnesium salts of unsaturated fatty acids having 3 to 8 carbon atoms (e.g., acrylic acid and methacrylic acid), with zinc acrylate being especially preferred. The amount of the co-crosslinking agent blended is 3 to 50 parts by weight, preferably 20 to 48 parts by weight per 100 parts by weight of the base rubber.

Examples of the inert filler include zinc oxide, barium sulfate, silica, calcium carbonate, and zinc carbonate, with zinc oxide and barium sulfate being commonly used. The amount of the filler blended is governed by the specific gravity of the core and the cover, the weight specification of the ball, etc. and not critical although it is usually 10 to 30 parts by weight per 100 parts by weight of the base rubber. It is understood that in the practice of the invention, the solid core is given an optimum hardness by properly adjusting the amount of zinc oxide and barium sulfate blended.

A solid core composition is prepared by kneading the above-mentioned components in a conventional mixer such as a Banbury mixer and roll mill, and it is compression or injection molded in a core mold. The molding is then cured into a solid core by heating at a sufficient temperature for the crosslinking agent and co-crosslinking agent to function (for example, about 130 to 170°C when dicumyl peroxide and zinc acrylate are used as the crosslinking agent and the co-crosslinking agent, respectively).

The solid core should have a distortion or deformation of at least 2.7 mm, preferably 2.9 to 7.0 mm, more preferably 3.0 to 6.0 mm under an applied load of 100 kg. A distortion of less than 2.7 mm under an applied load of 100 kg (hard core) would give disadvantages such as a hard hitting feel. A too much distortion (too soft core) would sometimes result in poor restitution.

The solid core preferably has a specific gravity of 0.9 to 1.2, more preferably 1.04 to 1.20, especially 1.05 to 1.18.

In the practice of the invention, the solid core preferably has a diameter of 30 to 40 mm, especially 33 to 39 mm. Also the solid core may be of multi-layer structure insofar as it satisfies the above-defined distortion under an applied load of 100 kg.

Next, the inner cover layer is formed mainly of a thermoplastic polyester elastomer.

The thermoplastic polyester elastomer used herein includes polyether ester type multi-block copolymers synthesized from terephthalic acid, 1,4-butane diol, and polytetramethylene glycol (PTMG) or polypropylene glycol (PPG) wherein polybutylene terephthalate (PBT) portions become hard segments and polytetramethylene glycol (PTMG) or polypropylene glycol (PPG) portions become soft segments, for example, Hytrel 3078, 4047, G3548W, 4767, and 5577 (by Toray duPont K.K.).

To the thermoplastic polyester elastomer, an ionomer resin having a Shore D hardness of at least 55, preferably 55 to 70, more preferably 56 to 69 can be added in a proportion of less than 70 parts by weight per 100 parts by weight of the thermoplastic polyester elastomer. In the event that the ionomer resin having a Shore D hardness of at least 55 is not contained in the outer cover layer to be described later, it is essential to mix the ionomer resin with the thermoplastic polyester elastomer. Preferably 3 to 70 parts by weight, more preferably 4 to 68 parts by weight of the ionomer resin is mixed per 100 parts by weight of the thermoplastic polyester elastomer.

Understandably, another polymer may be blended with the thermoplastic polyester elastomer insofar as the objects of the invention are not impaired.

Further the inner cover layer composed mainly of the thermoplastic polyester elastomer may contain 0 to about 30% by weight of an inorganic filler such as zinc oxide, barium sulfate, and titanium dioxide.

The inner cover layer should have a Shore D hardness of 28 to 58, especially 30 to 56. A Shore D hardness of less than 28 would detract from restitution whereas hitting feel would become too hard above 58.

Further, the inner cover layer should preferably have a specific gravity of 1.05 to 1.3, especially 1.06 to 1.2.

It is noted that the inner cover layer preferably has a gage of 0.5 to 3.0 mm, especially 1.0 to 2.5 mm.

On the other hand, the outer cover layer is formed of a thermoplastic polyurethane elastomer.

The thermoplastic polyurethane elastomer used herein has a molecular structure consisting of a high molecular weight polyol compound constituting a soft segment, a monomolecular chain extender constituting a hard segment, and a diisocyanate.

The high molecular weight polyol compound is not critical and may be any of polyester polyols, polyether polyols, copolyester polyols, and polycarbonate polyols. Exemplary polyester polyols include polycaprolactone glycol, poly(ethylene-1,4-adipate) glycol, and poly(butylene-1,4-adipate) glycol; an exemplary copolyester polyol is poly(diethylene glycol adipate) glycol; an exemplary polycarbonate polyol is (hexanediol-1,6-carbonate) glycol; and an exemplary polyether polyol is polyoxytetramethylene glycol. Their number average molecular weight is about 600 to 5,000, preferably 1,000 to 3,000.

As the diisocyanate, aliphatic diisocyanates are preferably used in consideration of the yellowing resistance of the cover. Examples include hexamethylene diisocyanate (HDI), 2,2,4- or 2,4,4-trimethylhexamethylene diisocyanate (TMDI), and lysine diisocyanate (LDI). HDI is especially preferred for its compatibility with another resin upon blending.

The monomolecular chain extender is not critical and may be selected from conventional polyhydric alcohols and amines. Examples include 1,4-butylene glycol, 1,2-ethylene glycol, 1,3-propylene glycol, 1,6-hexylene glycol, 1,3-butylene glycol, dicyclohexylmethylmethanediamine (hydrogenated MDA), and isophoronediamine (IPDA).

Of the thermoplastic polyurethane elastomers, those having a tans peak temperature of lower than -15°C, especially -16°C to -50°C as determined by viscoelasticity measurement are preferred in view of resiliency.

As the thermoplastic polyurethane elastomer, there may be used commercially available ones whose diisocyanate component is aliphatic, for example, Pandex T7298 (-20°C), T7295 (-26°C), and T7890 (-30°C) (by Dai-Nihon Ink Chemical Industry K.K.). Note that the numerals in parentheses each represent a tanδ peak temperature.

To the thermoplastic polyurethane elastomer, an ionomer resin having a Shore D hardness of at least 55, preferably 55 to 70, more preferably 56 to 69 can be added in a proportion of less than 70 parts by weight per 100 parts by weight of the thermoplastic polyurethane elastomer. In the event that the ionomer resin having a Shore D hardness of at least 55 is not contained in the aforementioned inner cover layer, it is essential to mix the ionomer resin with the thermoplastic polyurethane elastomer. Preferably 2 to 70 parts by weight, more preferably 3 to 68 parts by weight of the ionomer resin is mixed per 100 parts by weight of the thermoplastic polyurethane elastomer.

Understandably, another polymer may be blended with the thermoplastic polyurethane elastomer insofar as the objects of the invention are not impaired.

Further the outer cover layer composed mainly of the thermoplastic polyurethane elastomer may contain 0.5 to 30% by weight, especially 1 to 25% by weight of an inorganic filler such as zinc oxide, barium sulfate, and titanium dioxide.

The outer cover layer should have a Shore D hardness of 30 to 55, preferably 35 to 54, more preferably 38 to 53. A Shore D hardness of less than 30 would detract from restitution whereas hitting feel would become too hard above 55.

The outer cover layer should preferably have a specific gravity of 1.05 to 1.4, especially 1.08 to 1.3.

The outer cover layer preferably has a gage of 0.5 to 2.5 mm, especially 1.0 to 2.3 mm.

The inner and outer cover layers preferably have a total gage (overall cover gage) of 1.0 to 5.5 mm, more preferably 1.5 to 5.0 mm, especially 1.5 to 3.5 mm.

As mentioned above, it is essential in the practice of the invention to mix an ionomer resin having a Shore D hardness of at least 55 with the thermoplastic polyester elastomer and/or the thermoplastic polyurethane elastomer. Useful as the ionomer resin having a Shore D hardness of at least 55 are Himilan 1605 and Himilan 1706 by Mitsui duPont Polychemicals K.K. The mixing of the ionomer resin having a Shore D hardness of at least 55 is effective for maintaining a good balance of hardness and resiliency. In contrast, such effects are not achievable by mixing an ionomer resin having a Shore D hardness of lower than 55. The amount of the ionomer resin having a Shore D hardness of at least 55 blended is as described above while too large amounts prevent the elastomer from fully exerting its effect and too small amounts of the ionomer resin fail to achieve its addition effect.

Understandably, the inner and outer cover layers may be formed by well-known techniques such as injection molding and compression molding using half shells.

The multi-piece solid golf ball thus obtained should preferably have an inertia moment of at least 83 g-cm², especially 83.5 to 87.0 g-cm² as measured by the method described later. An inertia moment of less than 83 g-cm² would lead to the disadvantage that the ball rolling upon putting becomes unsustained.

The outer cover layer is formed with dimples in a conventional manner. With respect to the diameter, weight and other parameters, the golf ball of the invention is constructed in accordance with the Rules of Golf to a diameter of not less than 42.67 mm and a weight of not greater than 45.93 grams.

There has been described a multi-piece solid golf ball featuring an increased flight distance, superior control, pleasant feeling, and improved durability.

### EXAMPLE

Examples of the present invention are given below together with Comparative Examples by way of illustration and not by way of limitation.

### Examples and Comparative Examples

Solid cores of the composition shown in Table 1 were prepared.

**Table 1**

| Solid core composition (pbw) | Example | | | | | Comparative Example | | | | | |
|---|---|---|---|---|---|---|---|---|---|---|---|
| | 1 | 2 | 3 | 4 | 5 | 1 | 2 | 3 | 4 | 5 | 6 |
| Polybutadiene* | 100 | 100 | 100 | 100 | 100 | 100 | 100 | 100 | 100 | 100 | 100 |
| Dicumyl peroxide | 1.2 | 1.2 | 1.2 | 1.2 | 1.2 | 1.2 | 1.2 | 1.2 | 1.2 | 1.2 | 1.2 |
| Barium sulfate | 5 | 2.6 | 6.1 | 2.4 | 8.2 | 0 | 19 | 21.2 | 12.9 | 20.7 | 10 |
| Zinc oxide | 5 | 5 | 5 | 5 | 5 | 3.8 | 5 | 5 | 5 | 5 | 5 |
| Antioxidant | 0.2 | 0.2 | 0.2 | 0.2 | 0.2 | 0.2 | 0.2 | 0.2 | 0.2 | 0.2 | 0.2 |
| Zinc salt of pentachlorothiophenol | 1 | 1 | 1 | 1 | 1 | 1 | 1 | 1 | 1 | 1 | 1 |
| Zinc acrylate | 31.1 | 25.9 | 25.9 | 25.9 | 22.2 | 39.2 | 33.3 | 25.9 | 34 | 34 | 31.8 |

| | | | | | | | | | | | |
|---|---|---|---|---|---|---|---|---|---|---|---|
| * Polybutadiene: BR01 by Nippon Synthetic Rubber K.K. | | | | | | | | | | | |

Next, the cores each were enclosed with an inner cover layer of the composition shown in Table 2 by injection molding and then with an outer cover layer of the composition shown in Table 3 by injection molding, obtaining three-piece golf balls having a weight and diameter as shown in Tables 4 and 5. Compositions f,g,h in Table 2 and F,G,H,I in Table are not according to the invention and were tested for comparative purposes only.

The golf balls were examined for inertia moment, flight distance, spin rate, feeling, scraping resistance, and consecutive durability by the following tests. The results are shown in Tables 4, in accordance with the invention, and 5, showing the comparative examples.

### Inertia moment

It is calculated according to the equation shown below. More particularly, the inertia moment is a value calculated from the diameters (gages) and specific gravities of the respective layers and it can be determined from the following equation on the assumption that the ball is spherical. Although the ball is regarded spherical for the calculation purpose, the specific gravity of the outer cover layer is lower than the specific gravity of the outer cover-forming resin itself because the dimples are present on the actual ball. The specific gravity of the outer cover layer is herein designated a phantom outer cover layer specific gravity, which is used for the calculation of an inertia moment M.${\text{M = (π/5880000)x{(r1-r2)xD1}}^{\text{5}} {\text{+ (r2-r3)xD2}}^{\text{5}} {\text{+ r3xD3}}^{\text{5}} \text{}}$
M: inertia moment (g-cm²)
r1: core specific gravity
D1: core diameter
r2: inner cover layer specific gravity
D2: inner cover layer diameter (the diameter of a sphere obtained by forming the inner cover layer around the core)
r3: phantom outer cover layer specific gravity
D3: outer cover layer diameter (ball diameter)

Note that the diameters are expressed in mm.

### Flight distance

Using a swing robot, the ball was hit with a driver (#W1, head speed 45 m/sec.) to measure a carry and total distance.

### Spin rate

A spin rate was calculated from photographic analysis by photographing the behavior of the ball immediately after impact with #W1 and a sand wedge (#SW, head speed 20 m/sec.).

### Feeling

Three professional golfers actually hit the ball with #W1 and a putter (#PT) to examine the ball for feeling according to the following criteria.
- ○:: soft
- Δ:: somewhat hard
- ×:: hard

### Scraping resistance

Using the swing robot, the ball was hit at two points with a sand wedge (#SW, head speed 38 m/sec.). The ball at the hit points was visually examined.
- ○:: good
- Δ:: medium
- ×:: poor

### Consecutive durability

Using a flywheel hitting machine, the ball was repeatedly hit at a head speed of 38 m/sec. The ball was evaluated in terms of the number of hits repeated until the ball was broken.
○: good
×: poor

**Table 2**

| Inner cover layer (pbw) | Shore D | Specific gravity | a | b | c | d | e | f | g | h |
|---|---|---|---|---|---|---|---|---|---|---|
| Hytrel 3078 | 30 | 1.08 | - | - | - | 70 | 80 | - | - | - |
| Hytrel 4047 | 40 | 1.12 | 80 | - | 100 | - | - | - | - | - |
| Hytrel 4767 | 47 | 1.15 | - | 80 | - | - | - | - | - | - |
| PEBAX 3533 | 42 | 1.01 | - | - | - | - | - | 100 | - | - |
| Himilan 1605 | 61 | 0.94 | 10 | 10 | - | 15 | - | - | - | 50 |
| Himilan 1706 | 60 | 0.94 | 10 | 10 | - | 15 | - | - | 60 | 50 |
| Surlyn AM7317 | 63 | 0.94 | - | - | - | - | 10 | - | - | - |
| Surlyn AM7318 | 63 | 0.94 | - | - | - | - | 10 | - | - | - |
| Surlyn 8120 | 45 | 0.94 | - | - | - | - | - | - | 40 | - |
| Titanium dioxide | - | 4.2 | - | - | - | 20 | 10 | - | 5.13 | 5.13 |
| Hytrel: Toray duPont K.K., thermoplastic polyester elastomer | | | | | | | | | | |
| PEBAX 3533: Atochem, polyamide elastomer | | | | | | | | | | |
| Himilan: Mitsui duPont Polychemicals K.K., ionomer resin | | | | | | | | | | |
| Surlyn AM7317/AM7318/8120: E. I. duPont, ionomer resin | | | | | | | | | | |

**Table 3**

| Outer cover layer (pbw) | Shore D | Specific gravity | A | B | C | D | E | F | G | H | I |
|---|---|---|---|---|---|---|---|---|---|---|---|
| PANDEX T7890 | 39 | 1.16 | - | 80 | - | - | - | - | - | - | - |
| PANDEX T7295 | 46 | 1.16 | 100 | - | - | - | - | - | - | - | - |
| PANDEX T7298 | 50 | 1.16 | - | - | 95 | 100 | 90 | - | - | - | - |
| Himilan 1605 | 61 | 0.94 | - | 10 | 2.5 | - | - | - | 50 | - | - |
| Himilan 1706 | 60 | 0.94 | - | 10 | 2.5 | - | - | - | 50 | 40 | 70 |
| Surlyn AM7317 | 63 | 0.94 | - | - | - | - | 5 | - | - | - | - |
| Surlyn AM7318 | 63 | 0.94 | - | - | - | - | 5 | - | - | - | - |
| Surlyn 8120 | 45 | 0.94 | - | - | - | - | - | 100 | - | 60 | 30 |
| Titanium dioxide | - | 4.2 | 2.7 | 20 | 2.7 | 2.7 | 2.7 | 5.13 | 5.13 | 5.13 | 5.13 |
| PANDEX T7890/T7295/T7298: Dai-Nihon Ink Chemical Industry K.K., thermoplastic polyurethane elastomer | | | | | | | | | | | |
| Himilan: Mitsui duPont Polychemicals K.K., ionomer resin | | | | | | | | | | | |
| Surlyn AM7317/AM7318/8120: E. I. duPont, ionomer resin | | | | | | | | | | | |

**Table 4**

| | | Example | | | | |
|---|---|---|---|---|---|---|
| | | 1 | 2 | 3 | 4 | 5 |
| Core | Weight (g) | 28.66 | 26.14 | 25.51 | 27.90 | 28.49 |
| | Diameter (mm) | 36.60 | 35.80 | 35.30 | 36.60 | 36.60 |
| | Distortion @100kg (mm) | 3.30 | 4.00 | 4.00 | 4.00 | 4.50 |
| | Specific gravity | 1.116 | 1.088 | 1.108 | 1.087 | 1.110 |
| Inner cover layer | Type | a | b | c | d | e |
| | Shore D hardness | 45 | 51 | 40 | 41 | 38 |
| | Specific gravity | 1.08 | 1.10 | 1.12 | 1.18 | 1.13 |
| | Gage (mm) | 1.60 | 2.00 | 1.70 | 1.60 | 1.60 |
| Outer cover layer | Type | A | B | C | D | E |
| | Specific gravity | 1.18 | 1.26 | 1.17 | 1.18 | 1.16 |
| | Gage (mm) | 1.45 | 1.45 | 2.00 | 1.45 | 1.45 |
| | Shore D hardness | 46 | 44 | 51 | 50 | 52 |
| Ball | Weight (g) | 45.30 | 45.30 | 45.30 | 45.30 | 45.30 |
| | Diameter (mm) | 42.70 | 42.70 | 42.70 | 42.70 | 42.70 |
| Inertia moment (g-cm²) | | 84.2 | 85.2 | 84.4 | 85.0 | 84.3 |
| #W1/HS45 | Carry (m) | 208.9 | 209.0 | 208.7 | 208.8 | 208.5 |
| | Total (m) | 222.2 | 222.8 | 223.4 | 225.2 | 222.9 |
| | Spin (rpm) | 2938 | 2763 | 2761 | 2798 | 2702 |
| | Feeling | O | O | O | O | O |
| #SW/HS20 approach spin (rpm) | | 6273 | 6218 | 6108 | 6111 | 6095 |
| #PT feeling | | O | O | O | O | O |
| Scraping resistance | | O | O | O | O | O |
| Consecutive durability | | O | O | O | O | O |

**Table 5**

| | | Comparative Example | | | | | |
|---|---|---|---|---|---|---|---|
| | | 1 | 2 | 3 | 4 | 5 | 6 |
| Core | Weight (g) | 25.83 | 30.25 | 27.47 | 29.72 | 30.76 | 29.16 |
| | Diameter (mm) | 35.50 | 36.40 | 35.30 | 36.50 | 36.50 | 36.50 |
| | Distortion @100kg (mm) | 2.20 | 3.00 | 4.00 | 2.90 | 2.90 | 3.20 |
| | Specific gravity | 1.103 | 1.198 | 1.193 | 1.167 | 1.208 | 1.145 |
| Inner cover layer | Type | c | f | c | c | g | h |
| | Shore D hardness | 40 | 42 | 40 | 40 | 56 | 62 |
| | Specific gravity | 1.12 | 1.01 | 1.12 | 1.12 | 0.98 | 0.98 |
| | Gage (mm) | 1.63 | 1.80 | 1.70 | 1.60 | 1.60 | 1.60 |
| Outer cover layer | Type | D | F | G | H | I | D |
| | Specific gravity | 1.183 | 0.980 | 0.980 | 0.980 | 0.980 | 1.183 |
| | Gage (mm) | 1.98 | 1.35 | 2.00 | 1.50 | 1.50 | 1.50 |
| | Shore D hardness | 50 | 45 | 62 | 53 | 58 | 50 |
| Ball | Weight (g) | 45.30 | 45.30 | 45.30 | 45.30 | 45.30 | 45.30 |
| | Diameter (mm) | 42.70 | 42.70 | 42.70 | 42.70 | 42.70 | 42.70 |
| Inertia moment (g-cm²) | | 84.6 | 81.2 | 81.3 | 82.1 | 80.9 | 83.4 |
| #W1/HS45 | Carry (m) | 208.1 | 205.3 | 207.9 | 205.8 | 207.9 | 208.1 |
| | Total (m) | 217.2 | 217.5 | 221.0 | 218.1 | 219.2 | 220.3 |
| | Spin (rpm) | 3075 | 3001 | 2548 | 2898 | 2689 | 2734 |
| | Feeling | X | Δ | O | Δ | O | O |
| #SW/HS20 approach spin (rpm) | | 6251 | 6236 | 4923 | 6211 | 5632 | 6132 |
| #PT feeling | | O | O | X | O | X | X |
| Scraping resistance | | O | Δ | O | Δ | Δ | X |
| Consecutive durability | | O | O | X | O | O | X |

## Claims

1. A multi-piece solid golf ball comprising a solid core and a cover having an inner and an outer layer surrounding the core, **characterized in that** said solid core has a distortion of at least 2.7 mm under an applied load of 100 kg, said inner cover layer is formed mainly of a thermoplastic polyester elastomer, said outer cover layer is formed mainly of a thermoplastic polyurethane elastomer, one or more ionomer resins having a Shore D hardness of at least 55 are mixed with either one or both of the thermoplastic polyester elastomer of said inner cover layer and the thermoplastic polyurethane elastomer of said outer cover layer, said inner cover layer has a Shore D hardness of 28 to 58, and said outer cover layer has a Shore D hardness of 30 to 55.

2. The golf ball of claim 1 having the inner cover layer wherein the ionomer resin having a Shore D hardness of at least 55 is mixed in a proportion of 3 to 70 parts by weight per 100 parts by weight of the thermoplastic polyester elastomer.

3. The golf ball of claim 1 or 2 having the outer cover layer wherein the ionomer resin having a Shore D hardness of at least 55 is mixed in a proportion of 2 to 70 parts by weight per 100 parts by weight of the thermoplastic polyurethane elastomer.

4. The golf ball of any one of claims 1 to 3 wherein the ball as a whole has an inertia moment of at least 83 g-cm².

5. The golf ball of any one of claims 1 to 4 wherein 0.5 to 30% by weight of an inorganic filler is added to said outer cover layer.

6. The golf ball of any one of claims 1 to 5 wherein said inner cover layer contains 0 to 30% by weight of an inorganic filler.

7. The golf ball of any one of claims 1 to 6 wherein said outer cover layer has a specific gravity of 1.05 to 1.4.

8. The golf ball of any one of claims 1 to 7 wherein said inner cover layer has a specific gravity of 1.05 to 1.3.

9. The golf ball of any one of claims 1 to 8 wherein said core has a specific gravity of 0.9 to 1.2.

10. The golf ball of any one of claims 1 to 9 wherein said outer cover layer has a gage of 0.5 to 2.5 mm, said inner cover layer has a gage of 0.5 to 3.0 mm, and said cover has a total gage of 1.0 to 5.5 mm.

## Patentansprüche

1. Mehrteiliger massiver Golfball, der einen massiven Kern und eine Hülle umfaßt, die eine innere und eine äußere Schicht hat, die den Kern umschließen, **dadurch gekennzeichnet, daß** der massive Kern unter einer ausgeübten Belastung von 100 kg eine Verformung von wenigstens 2,7 mm hat, wobei die innere Hüllenschicht hauptsächlich aus einem thermoplastischen Polyester-Elastomer geformt wird, die äußere Hüllenschicht hauptsächlich aus einem thermoplastischen Polyurethan-Elastomer geformt wird, wobei ein oder mehrere Ionomerharze mit einer Shore-D-Härte von wenigstens 55 mit dem thermoplastischen Polyester-Elastomer der inneren Hüllenschicht oder dem thermoplastischen Polyurethan-Elastomer der äußeren Hüllenschicht oder beiden gemischt werden, wobei die innere Hüllenschicht eine Shore-D-Härte von 28 bis 58 hat und die äußere Hüllenschicht eine Shore-D-Härte von 30 bis 55 hat.

2. Golfball nach Anspruch 1, der die innere Hüllenschicht hat, bei der das Ionomerharz, das eine Shore-D-Härte von wenigstens 55 hat, in einem Verhältnis von 3 bis 70 Gewichtsteilen auf 100 Gewichtsteile des thermoplastischen Polyester-Elastomers gemischt wird.

3. Golfball nach Anspruch 1 oder 2, der die äußere Hüllenschicht hat, bei der das Ionomerharz, das eine Shore-D-Härte von wenigstens 55 hat, in einem Verhältnis von 2 bis 70 Gewichtsteilen auf 100 Gewichtsteile des thermoplastischen Polyurethan-Elastomers gemischt wird.

4. Golfball nach einem der Ansprüche 1 bis 3, bei dem der Ball als Ganzes ein Trägheitsmoment von wenigstens 83 gcm² hat.

5. Golfball nach einem der Ansprüche 1 bis 4, bei dem der äußeren Hüllenschicht 0,5 bis 30 Gewichtsprozent eines anorganischen Füllstoffs hinzugefügt werden.

6. Golfball nach einem der Ansprüche 1 bis 5, bei dem die innere Hüllenschicht 0 bis 30 Gewichtsprozent eines anorganischen Füllstoffs enthält.

7. Golfball nach einem der Ansprüche 1 bis 6, bei dem die äußere Hüllenschicht ein spezifisches Gewicht von 1,05 bis 1,4 hat.

8. Golfball nach einem der Ansprüche 1 bis 7, bei dem die innere Hüllenschicht ein spezifisches Gewicht von 1,05 bis 1,3 hat.

9. Golfball nach einem der Ansprüche 1 bis 8, bei dem der Kern ein spezifisches Gewicht von 0,9 bis 1,2 hat.

10. Golfball nach einem der Ansprüche 1 bis 9, bei dem die äußere Hüllenschicht eine Dicke von 0,5 bis 2,5 mm hat, die innere Hüllenschicht eine Dicke von 0,5 bis 3,0 mm hat und die Hülle eine Gesamtdicke von 1,0 bis 5,5 mm hat.

## Revendications

1. Une balle de golf solide en plusieurs pièces comprenant un noyau solide et un revêtement possédant une couche intérieure et extérieure entourant le noyau, **caractérisé en ce que** ledit noyau solide subit une distorsion d'au moins 2,7 mm lorsqu'une charge de 100 kg lui est appliquée, ladite couche de revêtement intérieure est principalement constituée d'un élastomère polyester thermoplastique, ladite couche de revêtement extérieure est principalement constituée d'un élastomère polyuréthane thermoplastique, une ou plusieurs résines ionomère possédant une dureté Shore D d'au moins 55 sont mélangées soit avec l'élastomère polyester thermoplastique de ladite couche de revêtement intérieure ou avec l'élastomère polyuréthane thermoplastique de ladite couche de revêtement extérieure soit avec les deux élastomères, ladite couche de revêtement intérieure possède une dureté Shore D de 28 à 58, et ladite couche de revêtement extérieure possède une dureté Shore D de 30 à 55.

2. La balle de golf de la revendication 1 possédant une couche de revêtement intérieure dans laquelle la résine ionomère possédant une dureté Shore D d'au moins 55 est mélangée dans une proportion de 3 à 70 parties en poids pour 100 parties en poids de l'élastomère polyester thermoplastique.

3. La balle de golf de la revendication 1 ou 2 possédant une couche de revêtement extérieure dans laquelle la résine ionomère possédant une dureté Shore D d'au moins 55 est mélangée dans une proportion de 2 à 70 parties en poids pour 100 parties en poids de l'élastomère polyuréthane thermoplastique.

4. La balle de golf selon une quelconque des revendications 1 à 3 dans laquelle la balle dans son ensemble possède un moment d'inertie d'au moins 83 g-cm².

5. La balle de golf selon une quelconque des revendications 1 à 4 dans laquelle 0,5 à 30% en poids d'une matière de charge inorganique est ajoutée à ladite couche de revêtement extérieure.

6. La balle de golf selon une quelconque des revendications 1 à 5 dans laquelle ladite couche de revêtement intérieure contient 0 à 30% en poids d'une matière de charge inorganique.

7. La balle de golf selon une quelconque des revendications 1 à 6 dans laquelle ladite couche de revêtement extérieure possède un poids spécifique de 1,05 à 1,4.

8. La balle de golf selon une quelconque des revendications 1 à 7 dans laquelle ladite couche de revêtement intérieure possède un poids spécifique de 1,05 à 1,3.

9. La balle de golf selon une quelconque des revendications 1 à 8 dans laquelle ledit noyau possède un poids spécifique de 0,9 à 1,2.

10. La balle de golf selon une quelconque des revendications 1 à 9 dans laquelle ladite couche de revêtement extérieure possède une épaisseur de 0,5 à 2,5 mm, ladite couche de revêtement intérieure possède une épaisseur de 0,5 à 3,0 mm, et ledit revêtement possède une épaisseur totale de 1,0 à 5,5 mm.
